

# UNITED STATES PATENT OFFICE.

WILLIAM W. HULSE AND BENJAMIN T. MCKAY, OF MANCHESTER,  
GREAT BRITAIN.

## IMPROVEMENT IN PROCESSES OF MAKING FLOOR-CLOTHS.

Specification forming part of Letters Patent No. 177,842, dated May 23, 1876; application filed  
March 29, 1876.

*To all whom it may concern:*

Be it known that we, WILLIAM WILSON HULSE and BENJAMIN THOMAS MCKAY, both of Manchester, in the county of Lancaster, Kingdom of Great Britain, have invented an Improved Process of Manufacturing Floor-Cloths, of which the following is a specification:

This invention relates to floor-cloth, suitable for covering floors, passages, or stairs. A fabric composed, principally, of wool, woolen, or worsted material, or materials containing wool and animal hair, is formed in a manner similar as when making paper. This fabric is saturated with drying-oil and body color. The face is charged or coated with a ground color, and canvas is cemented to the back. The fabric may be plain or ornamental, as in the case of other floor-cloths.

When carrying the invention into effect a selection may be made of thirty-six per cent. of moist cow-hair, twenty per cent. of wool-waste, twenty per cent. of old woolen carpets, twenty-four per cent. of old carpets containing wool and linen. The cow-hair is first washed in a rag-engine, the "roll" being so arranged as not to have a cutting action. When cleansed the hair is drained. The remaining materials should be free from dirt. The materials are placed in a rag-engine, and as the carpets containing linen usually require the most beating they are first placed in the engine, the cow-hair being put in last. The materials are beaten in this engine until sufficiently washed, and are then "let down" into a second rag-engine, in which the materials are reduced to a pulp. The pulp so formed is supplied to a paper-machine, wherein a web or sheet is formed, the operation being similar as when making paper, with the exception that the wire of the machine travels more slowly—say, for example, at about five feet per minute. The supply of pulp is so regulated as that the finished web shall have a thickness suitable for its destined use—say, for example, a thickness of about one-sixteenth of an inch. The heat of the drying-cylinders should be graduated, the first cylinder being unheated, or being only warmed, the last cylinder being heated to a temperature not exceeding about 300° Fahrenheit. The dry web

so formed is passed through a mixture of oil and color. A suitable mixture consists of forty pounds of color ground in a minimum of raw linseed-oil and one hundred and thirty pounds of boiled linseed-oil. In passing through this mixture the web should be immersed therein—say, for about three-quarters of a minute. The web is then passed between calender-rollers, which press the oil and color into the fabric. The ordinary calender of the paper-machine may be employed for this purpose. The fabric is then suspended in festoons within a stove or heated room until the charge of oil and color is sufficiently dry. About forty-eight hours time is generally sufficient for the fabric to remain in the stove. It is then covered with a coating of oil and color, which may be applied in any suitable manner. In the arrangement found to be suitable the fabric is drawn over an endless couch or apron and under and in contact with the edge of a "doctor" knife or blade. The mixture of oil and color is roughly applied to the upper surface of the fabric, over which it is spread and made even by the action of the doctor. The color to be used must be suitable to the desired color of the finished floor-cloth. The fabric is again stoved until sufficiently dry, when it is backed with canvas which has been prepared and coated with oil and color in the following manner: The canvas is first rolled, pressed, or calendered, so as to close the interstices, and is then coated on one side with a size consisting of boiled "Irish moss" and whiting. It is then dried or stoved, and again calendered. It is then coated on the sized side with a mixture of oil and color. The coating with size and color is effected in the same manner as when coating the aforesaid fabric. The canvas is then stoved a second time, and is again calendered.

A cement is prepared in the following manner: Raw linseed-oil is heated gradually to a temperature of about 400° Fahrenheit, and to each gallon are added four ounces of acetate of lead, and eight ounces of flake litharge, the mixture being agitated and maintained at about the same temperature for about twenty-four hours, more or less, until converted into a thick tenacious substance, resembling caout-

chouic, when it is discharged from the boiler. One part of the said substance is mixed in a suitable machine with about two parts of earthy matter or matters, such as whiting, ocher, or umber, heat being applied to soften the cement, if necessary. The aforesaid fabric and the prepared canvas are passed together between calender-rollers, the surfaces which have been coated with oil and color, as aforesaid, being outward, and constituting the face and back of the finished floor-cloth. As the fabric passes over a roller, table, or apron to the said calender, the surface which is to be united to the canvas is roughly supplied with the said cement, which is evenly spread upon the surface by means of a doctor. The canvas is led over the top calender-roller, and meets the fabric, and is firmly united therewith by the action of the said calender. It is advisable to heat the calender-rollers in order to soften the cement.

The said fabric may be printed or be ornamented in the usual manner, and after being dried, aged, and seasoned by exposure to the air for several weeks the floor-cloth is finished and is ready for use, the edges being suitably cut or trimmed before or after the said aging

process, or the fabric may be used as a floor-cloth in its plain or unprinted condition.

The proportions of the ingredients herein given, and the mixtures of oil and color and the cement, are given as examples for guidance, but may be varied to some extent without departing materially from the nature of our invention.

We claim as our invention—

The process, substantially as described, of manufacturing floor-cloth—that is to say, forming a web or sheet of fibrous material, in which the fibers are aggregated by pulping, applying a liquid or plastic composition to the web, uniting the same to a backing of canvas previously coated, and then passing the compound fabric between calendering and condensing rollers.

WILLIAM W. HULSE.  
B. T. MCKAY.

Witnesses as to W. W. HULSE:

EDWARD K. DUTTON,  
HUGH G. GRANT.

Witnesses as to B. T. MCKAY:

GEORGE CLARK,  
ROBERT SKINNER.